

## UNITED STATES PATENT OFFICE

HANS MENGELE, OF WIESBADEN, GERMANY, ASSIGNOR TO BYK-GULDENWERKE CHEMISCHE FABRIK AKTIENGESELLSCHAFT, OF BERLIN, GERMANY, A CORPORATION OF GERMANY

## PROCESS FOR TONING SILVER PICTURES

No Drawing. Application filed June 4, 1931, Serial No. 542,108, and in Germany June 5, 1930.

In order to obtain a so-called sepia tone on photographic silver pictures, heretofore toning baths have been used, which either contained gold or selenium as a tone giving substance. The material distinction of gold toning baths lies in the fact the former are much more expensive than the latter and contain the tone giving ingredient as cation or as complexes. Principally on account of the lower cost the selenium toning baths have a steadily increasing demand. If, however, in spite of this gold toning baths are still in use, this is due to the fact that selenium toning baths possess several disadvantages.

Mainly two groups of selenium toning baths must be distinguished, namely selenium toning baths, capable of toning all kinds of silver photographs including also such directly on a layer of silver bromide emulsions, i. e., without a preceding bleaching bath. These baths, however, affect—owing to their strong acid or alkaline reaction—the hands of the worker and also the emulsion very disadvantageously. The other kind of selenium toning baths, however, does not possess this fault, but on the other hand it does not tone pictures on highly ripened halogen silver emulsions, particularly silver bromide emulsions and cannot produce the desired sepia tone without a preceding bleaching bath.

It has now been found that a sepia toning bath can be obtained, which on the one hand does not influence the hands of the worker and the emulsion, and on the other hand tones pictures on silver bromide emulsions in one single working process, i. e. without a preceding bleaching bath. Such a bath which is the subject matter of this invention contains simultaneously a solution of selenious acid and one or more easily water soluble salts of the sulphocyanic acid. It has been found that any and all salts of sulphocyanic acid, which dissolve in water relatively easily are very useful in connection with solutions of selenious acid.

A photograph inserted in such a solution shows within a few minutes a perfect sepia tone. Contrary to most of the toning baths, a selenium toning bath according to the pres-

ent invention produces always the same tone of picture on the same kind of emulsion; whereas toning baths heretofore known give exceedingly varying results in colour.

The addition of an organic acid to the solution greatly enhances the life of the toning bath, therefore increasing its efficiency and also the number of pictures which can be handled by one and the same solution and bath without adversely influencing its other properties and qualifications. This feature is the more surprising, since the addition of organic acids to gold toning baths and the addition of salts of organic acids to other selenium toning baths has no stabilizing effect.

Another advantage of the tone bath according to the present invention is that it can be sold in powdered form, and when ready for use can be easily dissolved in a determined quantity of distilled water.

The following example is indicative of the features of my invention:

|                        | Grams |
|------------------------|-------|
| Ammonium sulphocyanide | 10    |
| Citric acid            | 1 75  |
| Selenious acid         | 0,5   |

are dissolved in 100 ccm. of distilled water; with this solution the photographs are then treated.

From the foregoing description of the preferred embodiment of the invention it will be noted that a composition is made which is highly efficient and easy to handle.

While one preferred embodiment of the invention has been disclosed it is evident that various changes as to materials have been made which are the equivalent of those used, without departing from the spirit and scope of the invention.

Having thus described the invention what I claim is:

1. A composition of matter for toning photographic pictures comprising a solution containing selenious acid and a water soluble salt of sulphocyanic acid.

2. A composition of matter for toning photographic silver containing pictures comprising a bath solution containing selenious acid, a water soluble salt of sulphocyanic acid.

and a weakly dissociated organic acid for increasing the efficiency of said acid and salt.

3. A toning bath for photographic pictures comprising a solution containing ammonium sulphocyanide, a weakly dissociated soluble organic acid, and selenious acid.

4. A toning bath for photographic pictures comprising an aqueous solution of ammonium sulphocyanide, citric acid, and selenious acid.

5. A toning bath for photographic pictures comprising an aqueous solution of a sulphocyanide, citric acid, and selenious acid.

6. A composition for use in a toning bath for photographic pictures comprising a water soluble salt of sulphocyanic acid, citric acid and selenious acid.

In testimony whereof I affix my signature.

HANS MENGELE.

20

25

30

35

40

45

50

55

60

65

60

65

68

68

68

68

68

68

68